

Oct. 27, 1964

H. L. HOOVER ETAL

3,154,425

TEMPERATURE STABLE ULTRASONIC DELAY LINES

Filed June 19, 1961

~~Fig. 1~~



INVENTORS

HERBERT L. HOOVER  
AND MARTIN E. NORDBERG

BY Clarence R. Petty, Jr.  
ATTORNEY

1

3,154,425  
TEMPERATURE STABLE ULTRASONIC  
DELAY LINES

Herbert L. Hoover and Martin E. Nordberg, Corning, N.Y., assignors to Corning Glass Works, Corning, N.Y., a corporation of New York

Filed June 19, 1961, Ser. No. 118,185  
11 Claims. (Cl. 106—53)

This invention relates to solid ultrasonic delay lines, and more particularly to an ultrasonic delay line embodying a glass delay medium that is temperature stable.

One application for ultrasonic delay lines is in the radar receiver art, for example in moving target indication (MTI) devices. In such a device, the delay line is used to delay one received echo or pulse for comparison with a succeeding echo or pulse in order to determine whether any change has occurred in the time of the received signal. Another application is to provide for information storage in digital computers.

Since the inception of solid ultrasonic delay lines for these and other applications, vitreous silica has enjoyed widespread use as the delay, or wave propagation, medium in such delay lines. Materials having a crystalline structure have been avoided essentially because of excessive acoustic loss due to scattering. In general, organic materials are characterized by a high degree of attenuation, that is, loss of signal amplitude during transmission through the delay medium. Large single crystals have been seriously considered but are undesirable because of the directional characteristic of their elastic properties. Among glasses, vitreous silica has been of particular interest because of its extremely low attenuation characteristic.

It has been observed, however, that this silica medium is characterized by a negative temperature coefficient of time delay for shear waves that is on the order of 80 parts per million per centigrade degree. It also has a negative temperature coefficient of acoustic attenuation that is on the order of 5 to 10% per centigrade degree. A co-pending application, S.N. 50,366, filed August 18, 1960, in the name of Jason H. Eveleth and having a common assignee, describes the adverse effects resulting from large temperature coefficients and one means of overcoming such effects.

In general, it has been necessary to package delay lines in temperature controlled cases, usually containing a heating element, to counteract the effects of significant temperature changes. The expense and inconvenience of such auxiliary packaging and heating equipment is undesirable in any application, but particularly so in mobile and/or compact equipment such as air-borne radar, computers, and the like.

Ideally, the temperature coefficient of time delay for a delay medium should approximate zero. However, small variations can be tolerated; thus glasses having temperature coefficients up to about 8 parts per million per centigrade degree in absolute magnitude are generally acceptable.

It is also important that the material have as low an attenuation as possible, preferably not over about  $8 \times 10^{-3}$  decibels per cycle as measured at frequencies above one megacycle per second. The attenuation in fused silicas may be as low as 1 to  $2 \times 10^{-4}$  decibels per cycle. However, most commercially available multi-component glasses have attenuations on the order of 10 to  $60 \times 10^{-3}$  decibels per cycle, which is much higher than desirable.

It is also desirable that a material for delay line media have a relatively low temperature coefficient of attenuation, and it retain a stable characteristic delay time on aging. The latter is referred to as temporal stability of delay time and usually requires that the life-time change

2

not exceed about 0.003%. For example, this is equivalent to about 0.001 microsecond in a thirty microsecond delay line.

It is a primary purpose of the present invention to provide improved solid ultrasonic delay lines employing glass as the delay medium. A further purpose is to obviate the deficiencies encountered in lines employing vitreous silica as the delay medium. A further purpose is to provide glass delay media having the acceptable acoustical characteristics outlined above. A specific purpose is to provide a delay line incorporating an alkali-lead-silicate glass as the time delay medium.

In accordance with our invention, a solid ultrasonic delay line comprises a delay medium composed of an alkali-lead-silicate glass, the composition of which consists essentially of heavy metal oxides equivalent to 20-50% PbO, alkali metal oxides equivalent to 4-20% K<sub>2</sub>O, and the remainder SiO<sub>2</sub>. In a preferred embodiment, the glass is essentially composed of K<sub>2</sub>O, PbO and SiO<sub>2</sub>, but, under certain circumstances, other oxides may be considered equivalents, and substituted therefor, as described in detail later.

The invention is further described with reference to the accompanying drawing, in which:

FIG. 1 is a schematic illustration of a delay line assembly, and

FIG. 2 is a graphical illustration of a family of



glasses having special utility in connection with the present invention.

A simple delay line assembly, as schematically illustrated in FIG. 1, includes a delay or transmission medium 10, transducer members 11 and 12, backing members 13 and 14, and electrical signal input and output circuits 15 and 16. Delay medium 10 may be of any conventional form such as an elongated cylinder, a disc, a polygonal plate or other known delay line medium geometry. It is molded from an alkali-lead-silicate glass, as hereafter described, and ground and polished in accordance with usual glass delay medium finishing procedures.

Transducers 11 and 12 are composed of a crystalline piezo-electric material, such as barium titanate or crystalline quartz. They are sealed to, or otherwise maintained in tight contact with, facets on the delay medium 10.

Backing members 13 and 14 are firmly attached to crystals 11 and 12, respectively. Circuits 15 and 16, shown diagrammatically, may include any of the various components that are conventionally associated with delay lines. A schematic illustration is employed inasmuch as the improvement provided by this invention relates specifically to the delay medium 10.

FIG. 2 graphically illustrates a family of



glasses which our research has shown to be particularly advantageous for the fabrication of delay lines. In this figure, the content of PbO in percent by weight is plotted along the vertical axis. The corresponding percentage by weight of K<sub>2</sub>O is plotted along the horizontal axis.

With the PbO and K<sub>2</sub>O content for any glass thus fixed, the SiO<sub>2</sub> content is determined by difference, viz., 100%—(percent PbO+percent K<sub>2</sub>O). In general, any glass falling within the rhombic area designated A will possess the satisfactory delay line properties outlined earlier. In other words, the glasses will have temperature coefficients of time delay not exceeding about 8 parts per million per centigrade degree over the temperature range of —40° C. to 100° C.; their signal attenuation will not exceed about  $8 \times 10^{-3}$  decibels per cycle; temporal stability will not exceed about 0.003%; and the temperature coefficient of attenuation will be relatively low. Line B,

traversing rhombic area A, represents glass compositions having essentially a zero temperature coefficient of time delay. These are preferred compositions in applications where maximum temperature stability is of prime importance.

We have further found that the PbO content of glasses as defined with reference to FIG. 2 may be partially substituted for by other heavy metal divalent oxides, in particular CdO and BaO, in amounts up to about 10%. Also, Bi<sub>2</sub>O<sub>3</sub> may be substituted in amounts up to about 20%. These substituents, in the amounts indicated, tend to decrease attenuation slightly and, in the glasses of higher lead content, slightly increase temporal stability. They tend to increase temperature coefficient of time delay, but this can be compensated for by an adjustment in the alkali content. In amounts above the indicated ranges, they have a generally adverse effect on acoustical properties. In general, other substituents or additives provide no acoustic advantage and may have an adverse effect, particularly with respect to attenuation. However, minor amounts of antimony oxide, as a fining agent, and other compatible glass forming oxides, such as boric oxide, may be used as glass melting aids.

Our studies have further shown that the degree of acoustic attenuation in a glass decreases as K<sub>2</sub>O is replaced by Na<sub>2</sub>O, particularly in glasses having a high total alkali metal oxide content. A minimum value is reached when about one quarter of the total alkali metal oxide content, by weight, is Na<sub>2</sub>O, that is the actual ratio of K<sub>2</sub>O:Na<sub>2</sub>O, by weight, is about 3:1. Thereafter the trend changes direction, that is the degree of attenuation becomes greater as the Na<sub>2</sub>O content in a glass is further increased. It exceeds the limit of 8 × 10<sup>-3</sup> decibels/cycle when the ratio of Na<sub>2</sub>O:K<sub>2</sub>O exceeds about 1, and, accordingly, such further substitution is undesirable.

Replacement of K<sub>2</sub>O with Na<sub>2</sub>O, and resultant formation of a mixed alkali glass, also increases temporal instability. This effect also peaks with increasing Na<sub>2</sub>O replacement, in this case with about 1/3 to 1/2 of the K<sub>2</sub>O replaced. The effect on temporal instability is more pronounced in glasses of high total alkali metal oxide content, and hence, mixed alkali is avoided in such glasses especially where stability is an important factor. It may be noted that similar effects are noted in substituting other alkali metal oxides for K<sub>2</sub>O, e.g. Na<sub>2</sub>O and Li<sub>2</sub>O in combination.

In general, substitution of Na<sub>2</sub>O for K<sub>2</sub>O without changing temperature coefficient may be on the basis of about 0.4:1 on a weight basis, that is about 0.4% of the former for 1% of the latter with SiO<sub>2</sub> also being adjusted to account for the difference. Correspondingly, Li<sub>2</sub>O may be substituted on the basis of about 0.3% by weight for 1% K<sub>2</sub>O. Rb<sub>2</sub>O may be substituted on the basis of about 2.4% Rb<sub>2</sub>O for 1% K<sub>2</sub>O, but is of little interest, in part because of economic considerations. The minimizing effect of such substitutions on attenuation permits an extension of the useful glass area to include the area designated by C in FIG. 2. In terms of percent by weight, the alkali metal oxide content equivalent to K<sub>2</sub>O may be 4 to 20%, the PbO (or equivalent) content 20 to 50% and the remainder essentially silica. The compositions will further correspond to the areas designated A and C in FIG. 2 with the K<sub>2</sub>O and PbO contents taken as K<sub>2</sub>O and PbO equivalents respectively. With less than 20% PbO, these glasses tend to lack chemical stability, and above about 50% PbO, their attenuation becomes too high.

Line B in FIG. 2 may be mathematically expressed by the formula:

$$PbO = 62 - \frac{15}{7} \left( K_2O + 2.5 Na_2O + 3 Li_2O + \frac{Rb_2O}{2.4} \right)$$

Within the rhombic area of useful glasses, the PbO content may vary by about ±2% from this line. Therefore,

the permissible PbO content, within the limits 20 to 50%, may be expressed as

$$(62 \pm 2) - \frac{15}{7} \left( K_2O + 2.5 Na_2O + 3 Li_2O + \frac{Rb_2O}{2.4} \right)$$

Alternatively, the alkali metal oxide content, in terms of K<sub>2</sub>O equivalent, may be expressed as

$$K_2O = \frac{7}{15} (62 \pm 2 - PbO)$$

the PbO being within the range 20 to 50%.

The present glass compositions are similar in type to known optical and art glasses. Accordingly, they may be melted in accordance with known methods of melting such prior glasses. Thus, they may be melted in a continuous optical glass melting unit delivering about 1200 lbs. per day. The melting temperature may be 1200-1400° C. and usual precautions as to purity in batch materials and melting practice will be observed.

The molten glass may be shaped into blanks having roughly the desired form and subsequently finished by the usual grinding and polishing procedures. Large shaped blanks may, of course, be cut to any desired shape. The blanks may be annealed in accordance with conventional optical glass practice. However, it has been found that temporal stability is markedly improved by a slow annealing rate to temperatures well below the usual minimum annealing temperature, that is the strain point of the glass.

The following table sets forth, by way of more specifically illustrating the invention, the compositions of certain glasses, in percent by weight as calculated from the batch composition, together with acoustic properties measured for these glasses:

Table

|                                                    | 1     | 2     | 3     | 4     | 5     | 6     | 7     | 8     |
|----------------------------------------------------|-------|-------|-------|-------|-------|-------|-------|-------|
| SiO <sub>2</sub> .....                             | 47    | 53    | 58.4  | 53    | 60    | 57.8  | 57.8  | 58    |
| PbO.....                                           | 45    | 40    | 30    | 34    | 30    | 20    | 10    | 18.7  |
| K <sub>2</sub> O.....                              | 8     | 4.5   | 9     | 3.2   | 5     | 10    | 10    | 14    |
| Na <sub>2</sub> O.....                             | 1.8   | 2.6   | 1.3   | 4     | 2.2   | 2.2   | ----- | ----- |
| Li <sub>2</sub> O.....                             | 0.7   | ----- | 0.5   | 1     | ----- | ----- | ----- | ----- |
| BaO.....                                           | ----- | 8.0   | ----- | ----- | ----- | ----- | ----- | 9.3   |
| CdO.....                                           | ----- | ----- | ----- | ----- | ----- | 10    | 20    | ----- |
| Bi <sub>2</sub> O <sub>3</sub> .....               | 0     | 0     | 0     | 3     | 7     | 5     | 8.1   | 5.9   |
| T.C.D. (× 10 <sup>-3</sup> /C.°).....              | 6     | 4     | 6     | 5.5   | 5     | 6.7   | 7.5   | 7.6   |
| α (× 10 <sup>-3</sup> db/cycle).....               | 0.3   | 0.6   | 36    | ----- | 33    | ----- | ----- | ----- |
| ΔD <sub>t</sub> (percent × 10 <sup>-3</sup> )..... | ----- | ----- | ----- | ----- | ----- | ----- | ----- | ----- |

In this table temperature coefficient of time delay is measured in parts per centigrade degree, and identified as T.C.D. Likewise, α identifies attenuation in decibels per cycle and ΔD<sub>t</sub> temporal instability in percent.

Glasses of Examples 1 and 2 are particularly suitable because of their low temporal instability as well as low attenuation and temperature coefficients. Examples 3 and 6 illustrate glasses having desirable properties except for temporal instability. Stability data for Examples 4, 5, 7, and 8 are not available. However, Examples 4 and 8 might be predicted to be acceptable, while Examples 5 and 7 would not be, owing to high Na<sub>2</sub>O contents. Each of the compositions omits a fining agent, and the addition of 0.5% Sb<sub>2</sub>O<sub>3</sub> is satisfactory for this purpose.

For present purposes, the temperature coefficient of time delay (T.C.D.) is an average value generally expressed as,

$$T.C.D. = \frac{1}{X_0} \cdot \frac{X_2 - Y_1}{T_2 - T_1}$$

T<sub>2</sub> and T<sub>1</sub> are temperatures in °C. at the extremes of a given temperature range, X<sub>2</sub> and X<sub>1</sub> are the time delays for the delay medium measured, with the medium at the corresponding temperature extremes, in microseconds, and X<sub>0</sub> is the time delay at an intermediate temperature.

In measuring values of T.C.D. for glasses, a rectangular bar of the glass, 1/4" x 1" x 4", is cut and carefully ground and polished. The bar is provided with parallel end facets, to which are sealed, e.g. with phenyl benzoate,

silica bars having piezoelectric transducers sealed to their ends. A shear wave is then propagated through the glass test bar in 20 megacycle per second pulses of one microsecond duration, and measurements of time delay are made at precisely regulated temperatures. In evaluating the present glass media, measurements were made over a range of  $-15^{\circ}\text{C}$ . to  $+60^{\circ}\text{C}$ .

Similar glass test specimens were employed for attenuation coefficient measurements. As indicated earlier, attenuation is an expression of the decrease in, or loss of, amplitude of an acoustical wave or vibration as it is propagated through a delay medium. In determining coefficient of attenuation, designated by  $\alpha$ , the relative decrease of the amplitude of the input and output signals is measured; this figure is divided by the product of the measured time of propagation through the bar and the frequency of the acoustical vibration to provide the characteristic attenuation per wave length of wave traverse.

Total attenuation is expressed as

$$A = \alpha \cdot f \cdot t$$

where  $\alpha$  is the attenuation coefficient,  $f$  is the vibration frequency of the propagated wave and  $t$  is the total delay time of the medium in microseconds. In turn the attenuation coefficient may conveniently be expressed as

$$\alpha = 20 \log_{10} \left( \frac{\text{amplitude}_0}{\text{amplitude}_1} \right)$$

where "amplitude<sub>0</sub>" is the wave amplitude at a given point and "amplitude<sub>1</sub>" is the wave amplitude at a point spaced one wave length along the axis of propagation. The coefficient then is in units of decibels per cycle.

Temporal instability,  $\Delta D_t$ , is the percent change in the characteristic delay time of a particular medium over some period of time. Usually this is specified in terms of an indefinitely long time and referred to as lifetime stability.

What is claimed is:

1. In a solid ultrasonic delay line, an alkali-lead-silicate glass delay line medium having a temperature coefficient of time delay not exceeding eight parts per million per  $^{\circ}\text{C}$ ., an attenuation not exceeding  $8 \times 10^{-3}$  decibels per cycle, and being composed of about 10-50% PbO, 0-10% CdO, 0-10% BaO, 0-20%  $\text{Bi}_2\text{O}_3$ , the total content of PbO, CdO, BaO and  $\text{Bi}_2\text{O}_3$  being about 20-50%, about 4-20%  $\text{K}_2\text{O}$  in which up to  $\frac{1}{2}$  of the  $\text{K}_2\text{O}$  may be substituted by at least 1 additional alkali metal oxide in the indicated amount selected from the group consisting of 0-4%  $\text{Na}_2\text{O}$ , 0-3%  $\text{Li}_2\text{O}$ , and 0-24%  $\text{Rb}_2\text{O}$ , and wherein the substitution is on the basis of 0.4 part  $\text{Na}_2\text{O}$  for one part  $\text{K}_2\text{O}$ , 0.3 part  $\text{Li}_2\text{O}$  for 1 part  $\text{K}_2\text{O}$  and 2.4 parts  $\text{Rb}_2\text{O}$  for 1 part  $\text{K}_2\text{O}$ , the content of recited heavy metal oxides varying in inverse manner with the content of

recited alkali metal oxides, and the balance of the composition being essentially silica.

5 2. A delay line in accordance with claim 1, wherein the composition of the delay medium falls within a rhombic area designated by A and C in FIG. 2 of the drawing.

3. A delay line in accordance with claim 1, wherein the delay medium has temperature coefficient of time delay that is essentially zero and a composition falling 10 on line B in FIG. 2.

4. A delay line in accordance with claim 1, wherein the delay medium has a lifetime temporal instability of not over 0.003%, consists essentially of  $\text{K}_2\text{O}$ , PbO and  $\text{SiO}_2$ , and has a composition within area A in FIG. 2.

15 5. A delay line in accordance with claim 1 wherein the composition of the delay medium includes up to 10% CdO.

6. A delay line in accordance with claim 1 wherein the composition of the delay medium includes up to 10%

20 BaO.

7. A delay line in accordance with claim 1 wherein the composition of the delay medium includes up to 20%  $\text{Bi}_2\text{O}_3$ .

25 8. A delay line in accordance with claim 1 wherein the composition of the delay medium includes at least two alkali metal oxides at least one of which is  $\text{K}_2\text{O}$  in an amount not less than one half the total alkali metal oxide content.

9. A delay line in accordance with claim 8 wherein 30 the  $\text{K}_2\text{O}$  content is about three times the remaining alkali metal oxide content.

10. A delay line in accordance with claim 1 wherein the composition of the delay line medium is such that the content of recited heavy metal oxides within the range 35 of 20-50% is equal to

$$(62 \pm 2) \text{ minus } \frac{15}{7} \left( \text{K}_2\text{O} + 2.5 \text{ Na}_2\text{O} + 3 \text{ Li}_2\text{O} + \frac{\text{Rb}_2\text{O}}{2.4} \right)$$

11. A delay line in accordance with claim 1 wherein 40 the composition of the delay line medium is such that the content of recited heavy metal oxides within the range of 20-50% is equal to

$$62 \text{ minus } 15/7 \left( \text{K}_2\text{O} + 2.5 \text{ Na}_2\text{O} + 3 \text{ Li}_2\text{O} + \frac{\text{Rb}_2\text{O}}{2.4} \right)$$

#### References Cited in the file of this patent

#### UNITED STATES PATENTS

|              |               |       |                |
|--------------|---------------|-------|----------------|
| 50 2,663,006 | Andersen      | ----- | Dec. 15, 1953  |
| 2,727,214    | McSkimin      | ----- | Dec. 13, 1955  |
| 2,736,714    | Tiede         | ----- | Feb. 28, 1956  |
| 2,762,713    | Davis et al.  | ----- | Sept. 11, 1956 |
| 2,964,414    | Dalton et al. | ----- | Dec. 13, 1960  |
| 3,051,915    | Hoover et al. | ----- | Aug. 28, 1962  |